

## UNITED STATES PATENT OFFICE

JOHN D. RUE, OF ASHEVILLE, NORTH CAROLINA, ASSIGNOR TO THE CHAMPION FIBRE COMPANY, OF CANTON, NORTH CAROLINA, A CORPORATION OF OHIO

## PROCESS FOR THE PURIFICATION OF CHEMICAL WOOD PULP

No Drawing.

Application filed August 20, 1928. Serial No. 300,961.

This invention relates to processes for the purification or refining of chemical fibrous pulps adapted for paper making; more especially, it is concerned with a process for production, from chemical wood pulps, including particularly pulps produced from coniferous woods by the sulfate or soda processes of pulp making, of a purified pulp product characterized by a combination of a high degree of softness, whiteness, strength, toughness, and resistance to such mechanical treatments as are commonly given to fibrous materials in the course of their preparation for the paper, or paper board, machine.

Sulfate pulps prepared from coniferous woods possess potentially exceptional strength and toughness but, in their unbleached state, they are brown in color. Moreover, the development of their strength and toughness normally is attained only by a simultaneous development of hardness in the resulting sheet, which quality of hardness tends to give the sheet a rigidity and rattle which for many purposes are undesirable. In addition, sulfate pulps from coniferous woods contain certain constituents, including coloring matters, which are difficultly removable by bleaching, and easily hydrolyzable celluloses which at least in part are removable by bleaching. The removal of these hydrolyzable celluloses from the pulps, while contributing to the softness thereof and of the resulting paper, greatly reduces the strength and toughness. As a result, it is possible by the usual methods to obtain a product having a high degree of relative whiteness only at the sacrifice of strength and toughness, or vice versa.

It is, of course, well known that treatment of chemical wood pulps with solutions of caustic alkalies effects the dissolution of a portion of the coloring matter, and of a large proportion of the more easily hydrolyzable celluloses of the pulps. One characteristic result of the action of such alkaline solutions on chemical wood pulps is an increase in content of alpha cellulose (i. e., of cellulose resistant to caustic potash). By various treatments with alkaline solutions it is possible to increase the alpha cellulose content from

about 85%—the normal alpha cellulose content of bleached chemical wood pulp,—to as much as 98%.

I have found that chemical wood pulps having an alpha cellulose content of more than approximately 94% are deficient in strength and toughness, although they may possess a desirable softness, relative whiteness, and resistance to mechanical treatment. That is to say, while these high alpha cellulose pulps are particularly suitable for use in preparing cellulosic solutions for the spinning trade and for preparing lacquers and the like, they may not be so desirable for use in paper making. On the other hand, pulps having an alpha cellulose content of less than approximately 88% are deficient in softness and in resistance to mechanical treatment.

An object of the present invention, therefore, is to provide a process of preparing from unbleached sulfate, or soda, pulp obtained from coniferous wood, a purified pulp characterized by having an alpha cellulose content of from about 88% to about 94%, and especially adapted for use in paper making by reason of its softness, whiteness, strength, toughness and resistance to mechanical treatment.

I have found that there are certain conditions as regards the concentration and temperature of the alkaline solution, and certain sequences in the operations of bleaching and alkaline treatment, by the observance of which purified alkaline (i. e., sulfate or soda) pulps having the aforesaid desirable characteristics and properties may be produced. As an entity, my process comprises the following sequence of operations:

Alkaline (i. e., sulfate, or soda) pulp is subjected to a preliminary treatment with an oxidizing bleaching agent under such conditions,—to be set out with greater particularity hereinafter,—as to represent what I term a "drastic" bleaching treatment; the resulting partially bleached pulp in aqueous suspension is separated from bleach residues by washing,—either without or preferably with addition of an acid or an acidic reducing agent in such amount as to bring the mixture of partially bleached pulp, bleach

65

60

65

70

75

70

80

85

80

85

85

90

95

95

100

residues and suspending liquid to an acidity represented by a pH value of from 2 to 4; with the partially bleached and washed pulp, suitably thickened,—e. g., to 15% to 30% 5 pulp substance, there is admixed a relatively concentrated solution of a strong alkali,—e. g., caustic soda,—in excess, in such amount and concentration as to give the resulting suspension an alkalinity equivalent to that of 10 a solution of caustic soda of from 5% to 12% strength, and a pulp concentration of from 5% to 10%; the resulting strongly alkaline mixture is brought to and maintained at a temperature of from 70° to 212° F., preferably at a temperature of about 125° F., for a 15 relatively short period of time,—e. g., 10 minutes to about 6 hours, but preferably for from about one-half hour to about one hour,—with agitation; thereafter the suspension is concentrated by separating from the treated 20 pulp fibers so much of the alkaline liquor as is readily separable in a draining or filtering operation, and the separated treated pulp is washed. The resulting suspension of separated, treated, pulp,—after an optional intermediate treatment with an acid or an acidic 25 reducing agent in an amount sufficient to give the suspension an acidity represented by a pH value of from 2 to 4, and washing,—is given a relatively mild bleaching treatment, 30 preferably at a 3% to 4% consistence, with an oxidizing bleaching agent; and the resulting suspension of finally bleached and treated pulp, either without or preferably with addition 35 of an acid or an acidic reducing agent in an amount sufficient to give the suspension an acidity represented by a pH value of from 2 to 4, is washed free of bleach residues.

By a "drastic bleaching treatment", as that 40 expression is used in the foregoing general discription, I mean such a treatment as effects the major portion of the bleaching action to which the alkaline pulp is to be subjected during the whole sequence of operations. For 45 this purpose, there is used at this stage at least 50%, and preferably from 75% to 85%, of the total oxidizing bleaching agent with which the pulp is to be treated. I prefer to effect this operation with a stock suspension of from 8% to 12% solids (dry weight), using therein a relatively strong solution or suspension of an oxidizing bleaching agent,—say, 14% of bleaching powder. This partial 50 bleach prior to the alkaline treatment is essential in the successful carrying out of my process; otherwise, excessive proportions of bleaching agent would be required in the subsequent stage or stages of bleaching, resulting in the production of by-products soluble 55 in alkaline solution.

In such a case, the alpha cellulose content of the fully bleached product would be lowered, and the pulp would be deficient in one or more of the properties, strength, softness 60 and toughness. It is to avoid such an effect

that I find it desirable to use in the preliminary bleaching stage from one-half to three-fourths or more of the total bleaching agent to be used. Carrying out said preliminary bleach at a stock consistence of between 8% and 12% promotes an economy in time and in heat, and as well improves the quality of the final product. 70

The adjustment of the pH value of the pulp suspensions to a pH between 2 and 4 by means of an acid or an acidic reducing agent prior to the various washing operations is a preferred procedure in that thereby there are caused to be more readily removable by washing those bleach residues and certain other materials which are detrimental to the strength of the final pulp product, particularly, when allowed to remain in the pulp during the final stages of bleaching. Incomplete removal of these residues and materials from the final bleach may result in loss of color and of strength to the final, dried, pulp product. Naturally, where the highest qualities are not demanded, a satisfactory product can be produced without resorting to one or more of the acidification steps above mentioned. 80 85 90

Among operable acidic reducing agents are included sulfur dioxide, a solution containing stannous chloride in hydrochloric acid, or the like. The use of acidic reducing agents in removing bleach residues and the like from bleached pulp is described and claimed generally in the co-pending application Ser. No. 289,636, filed June 30, 1928. 95

Any other strong alkali may be substituted for the preferred caustic soda in the alkaline treatment stage of the process; provided the quantity and proportion used are chemically equivalent to the caustic soda solution specified herein. As stated previously, the caustic soda solution should have a concentration of between 5% and 12% after the partially bleached pulp has been suspended in it. The reaction between pulp and alkali should take place at a temperature between approximately normal room temperature,—say 70° F.,—and the boiling point of water; preferably, at about 125° F. Although no appreciable harm is done to the final pulp product if the alkaline treatment is prolonged for from 4 to 6 hours, the preferred period is one hour, and may be as short as from 10 to 15 minutes. 100 105 110 115

In treatment with caustic alkali of high concentration, the said caustic alkali has, in addition to its solvent action, the potential property of developing in the pulp a condition of hydration by reason of which the pulp swells while in contact with the solution, or with water, and shrinks when it is allowed to dry. The extent of the swelling and shrinking effects the curling and twisting of the fiber, with the result that the so-treated pulp may become exceptionally soft and bulky. Furthermore, the solvent effect may be such that the alpha cellulose content is in- 120 125 130

creased to a degree that the pulp no longer has strength and toughness, though its resistance to mechanical treatment may be high. Those effects are accentuated by lowering the temperature. I have found that by selecting a concentration between 5% and 12% and a temperature between 70° F. and 212° F., in suitable combinations, a pulp having the specified favorable qualities for paper making can be obtained.

An advantage of the process herein described and defined in the appended claims consists in this, that the use of an excess of strong alkali in the alkaline treatment stage permits the re-use of the separated alkaline liquor, after appropriate fortification with solid caustic or with a highly concentrated solution of caustic, in the treatment of a subsequent charge of pulp.

The following is a specific example illustrative of the process according to the present invention:

Unbleached pulp made by cooking pine wood by the sulfate process is semi-bleached at approximately 8% consistence at about 100° F., with approximately 14% of bleaching powder. The semi-bleached pulp is acidified to a pH value of approximately three, and thoroughly washed. Sufficient caustic soda and water are then added to the pulp to bring the pulp to approximately 5% consistence with a 6.5% solution of the caustic soda. The mass is agitated for approximately one hour at 125° F., drained, washed, acidified with  $\text{SO}_2$  to a pH value of approximately three, thoroughly washed.

The following properties are typical of a pulp prepared according to the above specific process:

An alpha cellulose content of 91.7%; a color, as measured upon an Ives tint photometer, of 80 parts red, 80 parts green and 75 parts blue; a maximum bursting strength of 270 after 220 minutes in the pebble mill and, as average values over the period of 190 to 340 minutes in the pebble mill, a bursting strength of 249; a folding endurance of 82; a tearing force of 6.5; and, in its preparation, a total bleach requirement of 16%.

By comparison, the following properties are typical of a pulp prepared from the same type of sulfate pulp by the ordinary process of purification. The data are expressed in the same arbitrary units as were the properties for the pulp prepared by the aid of my process: an alpha cellulose content of 80.8%; a color of 73 parts red, 70 parts green and 63 parts blue. The pulp after 200 minutes in the pebble mill was so thoroughly hydrated that it was practically impossible to prepare

sheets of paper from it. The total bleach required was 20.9%.

No means are at hand for expressing mathematically the degree of softness of pulps. As judged by the papermaker, the pulp prepared by my process is very much softer than are the pulps commonly prepared from equivalent impure chemical pulps.

I claim:

1. In purifying unbleached chemical wood pulp, the sequence of operations which comprises partially bleaching the pulp, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from about 10 minutes to about 6 hours, separating caustic alkali solution from the so-treated pulp and washing the latter, subjecting the treated and washed pulp to a second stage of bleaching treatment, and washing the resulting finally bleached pulp.

2. In purifying unbleached chemical wood pulp, the sequence of operations which comprises partially bleaching the pulp, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from about 10 minutes to about 6 hours and at a temperature greater than normal room temperature but less than the boiling point of water, separating caustic alkali solution from the so-treated pulp and washing the latter, subjecting the treated and washed pulp in aqueous suspension to a second stage of bleaching treatment, thereafter adjusting the acidity of the resulting suspension to a pH value of from 2 to 4, and washing the resulting finally bleached pulp.

3. In purifying unbleached chemical wood pulp, the sequence of operations which comprises partially bleaching the pulp, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from

about 10 minutes to about 6 hours and at a temperature greater than normal room temperature but less than the boiling point of water, separating caustic alkali solution from the so-treated pulp and washing the latter, adjusting the acidity of the resulting washed pulp to a pH value of from 2 to 4 and again washing the pulp, subjecting the treated and washed pulp in aqueous suspension to a second stage of bleaching treatment, thereafter adjusting the acidity of the resulting suspension to a pH value of from 2 to 4, and washing the resulting finally bleached pulp.

4. In purifying unbleached chemical wood pulp, the sequence of operations which comprises partially bleaching the pulp, adjusting the acidity of the resulting partially bleached pulp to a pH value of from 2 to 4, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from about 10 minutes to about 6 hours and at a temperature greater than normal room temperature but less than the boiling point of water, separating caustic alkali solution from the so-treated pulp and washing the latter, adjusting the acidity of the resulting washed pulp to a pH value of from 2 to 4 and again washing the pulp, subjecting the treated and washed pulp in aqueous suspension to a second stage of bleaching treatment thereafter adjusting the acidity of the resulting suspension to a pH value of from 2 to 4, and washing the resulting finally bleached pulp.

5. In purifying unbleached pulp prepared from coniferous wood by an alkaline process, the sequence of operations which comprises partially bleaching the pulp, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from about 10 minutes to about 6 hours and at a temperature greater than the normal room temperature but less than the boiling point of water, separating caustic alkali solution from the so-treated pulp and washing the latter, subjecting the treated and washed pulp in aqueous suspension to a second stage of bleaching treatment, thereafter adjusting the acidity of the resulting suspension to a pH value of

from 2 to 4, and washing the resulting finally bleached pulp.

6. In purifying unbleached pulp prepared from coniferous wood by the sulfate process, the sequence of operations which comprises partially bleaching the pulp, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from about 10 minutes to about 6 hours and at a temperature greater than normal room temperature but less than the boiling point of water, separating caustic alkali solution from the so-treated pulp and washing the latter, subjecting the treated and washed pulp in aqueous suspension to a second stage of bleaching treatment, thereafter adjusting the acidity of the resulting suspension to a pH value of from 2 to 4, and washing the resulting finally bleached pulp.

7. In purifying unbleached chemical wood pulp, the sequence of operations which comprises partially bleaching the pulp, washing the partially bleached pulp, treating the partially bleached and washed pulp with a solution of caustic alkali, the washed pulp and caustic alkali solution being brought together in such amounts and concentrations as to give a resulting suspension having an alkalinity equivalent to that of a caustic soda solution of from 5% to 12% strength and a pulp concentration of from about 5% to 10%, at a temperature above 70° but not in excess of 212° F., for from about one-half hour to about one hour, separating caustic alkali solution from the so-treated pulp and washing the latter, adjusting the acidity of the resulting washed pulp to a pH value of from 2 to 4 and again washing the pulp, subjecting the treated and washed pulp in aqueous suspension to a second stage of bleaching treatment, thereafter adjusting the acidity of the resulting suspension to a pH value of from 2 to 4, and washing the resulting finally bleached pulp.

8. In purifying unbleached chemical wood pulp, the sequence of operations which comprises partially bleaching the pulp, washing the partially bleached pulp, and thickening the same to from 15% to 30% pulp substance, treating the partially bleached and washed pulp with a solution of caustic alkali, the washed pulp and caustic alkali solution being brought together in such amounts and concentrations as to give a resulting suspension having an alkalinity equivalent to that of a caustic soda solution of from 5% to 12% strength and a pulp concentration of from

- about 5% to 10%, at a temperature of about 125° F., for from about one-half hour to about one hour, separating caustic alkali solution from the so-treated pulp and washing the latter, adjusting the acidity of the resulting washed pulp to a pH value of from 2 to 4 and again washing the pulp, subjecting the treated and washed pulp in aqueous suspension at a stock consistence of from 3% to 4% to a second stage of bleaching treatment, thereafter adjusting the acidity of the resulting suspension to a pH value of from 2 to 4, and washing the resulting purified pulp. 70
- 10 11. Process which comprises subjecting unbleached sulfate pulp obtained from coniferous wood at a suspension consistence of about 8% to a preliminary bleaching treatment with approximately 14% of bleaching powder based upon the weight of the dry pulp substance at about 100° F., acidifying the pulp suspension to a pH value of about 3, washing the so-acidified pulp and suitably thickening the same, admixing therewith caustic soda solution in such amount and concentration as to bring the resulting mixture to a consistence of approximately 5% of dry pulp substance with an alkalinity of the resulting solution equivalent to 6.5% of caustic soda, maintaining the mixture at about 125° F. for about 1 hour with agitation, draining caustic soda solution from the pulp in said mixture and washing the pulp, acidifying the pulp to a pH value of about 3 and again washing the pulp, subjecting the resulting pulp in an aqueous suspension containing about 4% of dry pulp substance to treatment with about 4% of bleaching powder based upon the weight of the dry pulp substance, thereafter acidifying the pulp suspension to a pH value of about 3, and washing the resulting so-acidified and finally bleached pulp. 75
- 15 12. In testimony whereof, I affix my signature. 105  
JOHN D. RUE. 105
- 20 13. 110
- 25 14. 115
- 30 15. 120
- 35 16. 125
- 40 17. 130
- 45 18. 135
- 50 19. 140
- 55 20. 145
- 60 21. 150
- 65 22. 155
- 70 23. 160
- 75 24. 165
- 80 25. 170
- 85 26. 175
- 90 27. 180
- 95 28. 185
- 100 29. 190